

Patented June 4, 1940

2,203,649

Br. 51/325

## UNITED STATES PATENT OFFICE

2,203,649

## ACID SOLUTION

Pieter Frederik Felkers, Dordrecht, Netherlands,  
assignor to Stikstofbindingsindustrie "Nederland"  
N. V., Kilkade, Zeehaven, Dordrecht,  
Netherlands

No Drawing. Application July 23, 1938, Serial  
No. 221,009. In the Netherlands July 28, 1937

6 Claims. (Cl. 148-8)

This invention relates to the art of pickling metals and more especially to means for improving the results obtained with acid pickling baths and for preventing the attack of metals by solutions of acid reaction.

It is well known that metals and metal alloys are attacked by organic and inorganic acids in the presence of water and especially by aqueous solutions of acids. In the pickling of metals with aqueous solutions of acids or acid salts, in order to remove scale and impurities on the surface of the treated metals, not only the scale and impurities are removed; a certain amount of the metal also dissolves under the formation of metal-salts in the bath, involving a loss of active acid.

One object of the invention is to prevent or minimize the dissolution of metal during pickling and the loss of active acid.

Another object of the invention is to prevent the attack of metals by acidic solutions in chemical and physical processes wherein such acidic solutions are used in metallic receptacles.

Another object is to prevent or minimize the contamination of the air with acid particles originating from the bath and carried into the atmosphere by the hydrogen generated during the pickling treatment, the presence of acid particles in the atmosphere being noxious for the workmen.

Still another object in view is to prevent or minimize the occurrence of gas enclosures in the treated metallic object, such enclosures of gas occurring frequently after pickling processes and being probably due to the solution of hydrogen gas developed by the process in the metallic surface.

A further object of the invention is to prevent or minimize the brittleness of the treated metal which is usually caused by pickling treatment, caused by the hydrogen "in statu nascendi" developed in the treatment.

Various compositions may be used for the purposes aforesaid, as will be described hereinafter.

According to the invention a non-oxidizing acid solution is used with an addition of an inhibitor of the group constituted by the alkyl-thiocyanates and the aralkylthiocyanates.

The addition of a small amount of these thiocyanates exerts a beneficial action on the pickling treatment and the above mentioned advantages are obtained when using an acid bath to which such compound is added.

Organic non-oxidizing acids, such as formic, acetic and oxalic acid may be successfully used. As a rule it will however be preferable to use a non-oxidizing mineral acid such as sulphuric and hydrochloric acid as the acid compound for the purpose in view, though other mineral or organic acids than those above mentioned and aqueous solutions of acid salts, such as sodium bisulfate may be profitably used.

Inhibitors, which appeared to be useful according to this invention are e. g. methylthiocyanate, benzylthiocyanate, dithiocyanato-ethane ( $\text{NCS}-\text{CH}_2-\text{CH}_2-\text{SCN}$ ), and other alkyl- or aralkylthiocyanates.

In certain cases the protecting action of the thiocyanate contained in the pickling baths can be improved by the addition of capillary active agents, such as wetting agents, and/or foaming agents and/or another inhibitor to the composition. Saponine has been found to be a useful addition.

The addition of an inhibitor other than a thiocyanate, for instance thiocarbamide, appears to improve the inhibiting action of the thiocyanate and also the inhibiting action of the additional inhibitor.

The thiocyanates have been found to also improve the properties of protective coatings serving to prevent corrosion of metals.

As an illustration of the invention some examples are given hereunder, wherein the results of tests with small pieces of hoop-iron are given.

The examples serve to elucidate and clarify the invention; the invention is however not restricted to the compositions and compounding substances mentioned therein.

The dimensions of the iron pieces were about 4.0 to 2.5 to 0.1 cm., their weight averaged 5-6 grams. The pieces were immersed in the solutions and under the conditions mentioned in the examples.

In all examples 100 ccms. of a 20% acid were used.

## Example 1

| Acid               | $\text{H}_2\text{SO}_4$ | $\text{H}_2\text{SO}_4$<br>0.033 gr. benzylthiocyanate. |
|--------------------|-------------------------|---------------------------------------------------------|
| Addition           |                         |                                                         |
| Temperature        | 80° C.                  | 80° C.                                                  |
| Reaction time      | 90 min.                 | 90 min.                                                 |
| Decrease of weight | 29.54%                  | 0.07%                                                   |
| Impeding action    |                         | 99.9%.                                                  |

## Example II

|                         |          |                             |
|-------------------------|----------|-----------------------------|
| Acid.....               | HCl..... | HCl.....                    |
| Addition.....           |          | 0.100 gr. hexylthiocyanate. |
| Temperature.....        | 30° C.   | 30° C.                      |
| Reaction time.....      | 90 min.  | 90 min.                     |
| Decrease of weight..... | 25.6%    | 0.073%                      |
| Impeding action.....    |          | 99.6%                       |

## Example III

|                         |          |                              |
|-------------------------|----------|------------------------------|
| Acid.....               | HCl..... | HCl.....                     |
| Addition.....           |          | 0.100 gr. benzylthiocyanate. |
| Temperature.....        | 30° C.   | 30° C.                       |
| Reaction time.....      | 90 min.  | 90 min.                      |
| Decrease of weight..... | 25.0%    | 0.059%                       |
| Impeding action.....    |          | 99.8%                        |

## Example IV

|                         |                                      |                                      |
|-------------------------|--------------------------------------|--------------------------------------|
| Acid.....               | H <sub>2</sub> SO <sub>4</sub> ..... | H <sub>2</sub> SO <sub>4</sub> ..... |
| Addition.....           |                                      | 0.100 gr. methylthiocyanate.         |
| Temperature.....        | 78° C.                               | 78° C.                               |
| Reaction time.....      | 90 min.                              | 90 min.                              |
| Decrease of weight..... | 77.5%                                | 0.141%                               |
| Impeding action.....    |                                      | 99.8%                                |

## Example IX

|                         |          |                              |
|-------------------------|----------|------------------------------|
| Acid.....               | HCl..... | HCl.....                     |
| Addition.....           |          | 0.040 gr. benzylthiocyanate. |
| Temperature.....        | 40° C.   | 40° C.                       |
| Reaction time.....      | 90 min.  | 90 min.                      |
| Decrease of weight..... | 10.90%   | 0.063%                       |
| Impeding action.....    |          | 99.4%                        |

## Example X

|                         |                                      |                                      |                                      |
|-------------------------|--------------------------------------|--------------------------------------|--------------------------------------|
| Acid.....               | H <sub>2</sub> SO <sub>4</sub> ..... | H <sub>2</sub> SO <sub>4</sub> ..... | H <sub>2</sub> SO <sub>4</sub> ..... |
| Addition.....           |                                      | 0.025 gr. benzylthiocyanate.         | 0.025 gr. Dr. Vogel's Beiz-Zusatz.   |
| Temperature.....        | 78° C.                               | 78° C.                               | 78° C.                               |
| Reaction time.....      | 90 min.                              | 90 min.                              | 90 min.                              |
| Decrease of weight..... | 56.20%                               | 0.11%                                | 27.7%                                |
| Impeding action.....    |                                      | 99.8%                                | 50.7%                                |

The superior results and superior inhibiting effect obtained by the composition according to this invention is illustrated by the comparative tests reproduced in the following table:

Table

|                                    |          |                                |                                |                                 |                                                       |                           |
|------------------------------------|----------|--------------------------------|--------------------------------|---------------------------------|-------------------------------------------------------|---------------------------|
| 30 Acid.....                       | HCl..... | HCl.....                       | HCl.....                       | HCl.....                        | HCl.....                                              | HCl.....                  |
| Addition.....                      |          | 0.100% Rodine 40. <sup>1</sup> | 0.100% Rodine 41. <sup>1</sup> | 0.100% Dr. Vogel's Beiz-Zusatz. | 0.100% Ferrophil <sup>1</sup> Extrem-Sparbeiz-Zusatz. | 0.080% benzylthiocyanate. |
| Temperature.....                   | 43° C.   | 43° C.                         | 43° C.                         | 43° C.                          | 43° C.                                                | 43° C.                    |
| Reaction time.....                 | 90 min.  | 90 min.                        | 90 min.                        | 90 min.                         | 90 min.                                               | 90 min.                   |
| Decrease of weight in percent..... | 12.45.   | 3.10.                          | 3.02.                          | 1.25.                           | 1.23.                                                 | 0.07.                     |
| Impeding action in percent.....    | 75.1.    | 75.7.                          | 90.0.                          | 90.1.                           | 90.4.                                                 | 35                        |

<sup>1</sup> Made by American Chemical Paint Co.

<sup>2</sup> Made by "Chemos" A. G., Aussig, Czechoslovakia.

## Example V

|                         |                                      |                                      |
|-------------------------|--------------------------------------|--------------------------------------|
| 45 Acid.....            | H <sub>2</sub> SO <sub>4</sub> ..... | H <sub>2</sub> SO <sub>4</sub> ..... |
| Addition.....           |                                      | 0.100 gr. dithiocyanethane.          |
| Temperature.....        | 78° C.                               | 78° C.                               |
| Reaction time.....      | 90 min.                              | 90 min.                              |
| Decrease of weight..... | 77.5%                                | 0.650%                               |
| Impeding action.....    |                                      | 99.2%                                |

## Example VI

|                         |                                      |                                      |
|-------------------------|--------------------------------------|--------------------------------------|
| 50 Acid.....            | H <sub>2</sub> SO <sub>4</sub> ..... | H <sub>2</sub> SO <sub>4</sub> ..... |
| Addition.....           |                                      | 0.025 gr. benzylthiocyanate.         |
| Temperature.....        | 78° C.                               | 78° C.                               |
| Reaction time.....      | 90 min.                              | 90 min.                              |
| Decrease of weight..... | 77.5%                                | 0.171%                               |
| Impeding action.....    |                                      | 99.8%                                |

## Example VII

|                         |                                      |                                      |
|-------------------------|--------------------------------------|--------------------------------------|
| 55 Acid.....            | H <sub>2</sub> SO <sub>4</sub> ..... | H <sub>2</sub> SO <sub>4</sub> ..... |
| Addition.....           |                                      | 0.0125 gr. benzylthiocyanate.        |
| Temperature.....        | 78° C.                               | 78° C.                               |
| Reaction time.....      | 90 min.                              | 90 min.                              |
| Decrease of weight..... | 77.5%                                | 0.240%                               |
| Impeding action.....    |                                      | 99.7%                                |

## Example VIII

|                         |          |                          |
|-------------------------|----------|--------------------------|
| 60 Acid.....            | HCl..... | HCl.....                 |
| Addition.....           |          | 0.010 gr. thiocarbamide. |
| Temperature.....        | 45° C.   | 45° C.                   |
| Reaction time.....      | 90 min.  | 90 min.                  |
| Decrease of weight..... | 16.25%   | 0.00%                    |
| Impeding action.....    |          | 100.0%                   |

Various changes may be made in the details disclosed in the foregoing specification without departing from the invention or sacrificing the advantages thereof.

I claim:

1. As a new pickling bath, an aqueous solution containing a substance of the group constituted by non-oxidizing acids and non-oxidizing acid salts and a substance of the group constituted by the alkylthiocyanates and the aralkylthiocyanates.

2. The pickling bath of claim 1, in which the acid belongs to the group constituted by sulphuric and hydrochloric acids.

3. The pickling bath of claim 1, in which the acid belongs to the group constituted by acetic, citric and oxalic acids.

4. The pickling bath of claim 1, in which the thiocyanate belongs to the group constituted by benzylthiocyanate, methylthiocyanate, dithiocyanethane.

5. As a pickling bath, an aqueous solution containing a substance of the group constituted by non-oxidizing acids and acid salts, a substance of the group constituted by the alkylthiocyanates and the aralkylthiocyanates, with an addition of thiocarbamide.

6. The process which consists in pickling metal with an aqueous solution containing a substance of the group consisting of non-oxidizing acids and acid salts and a substance of the group consisting of the alkylthiocyanates and the aralkylthiocyanates.

PIETER FREDERIK FELKERS.